

## UNITED STATES PATENT OFFICE

2,281,401

## LUBRICATING OIL COMPOSITION

Chester E. Wilson, San Pedro, Calif.

No Drawing. Application November 21, 1939,  
Serial No. 305,496

17 Claims.

(Cl. 252—32)

This invention relates to mineral lubricating oils which have been modified by the addition of constituents to impart to them special characteristics especially adapting them to severe service uses such as are encountered in Diesel engines, high output aviation engines and the like. This application is a continuation-in-part of my pending application, Serial No. 277,677, entitled "Modified lubricating oils."

In Diesel and similar engines the high temperatures developed in the cylinders tend to act upon lubricating oils to cause the deposition of resinous and varnish-like products on the pistons and elsewhere to produce lacquer-like coatings and carbonaceous materials, which tend to cause ring and valve sticking and interfere with engine operation. Furthermore, fuel residues from incomplete combustion of fuel contribute to the deposition of lacquer-like and carbonaceous materials in the engine. Previously in an effort to overcome these difficulties various types of metal soaps of fatty acids and the like have been introduced into the lubricating oil, and they have exhibited a detergent effect in that they have acted to prevent such depositions. However, in general, it has been observed that in those engines fitted with certain types of bearings, such as cadmium-silver or copper-lead bearings, the use of such fatty acid soap-compounded oils has often given rise to bearing corrosion, such corrosion apparently being due to the formation in the oil of corrosive materials of acidic character. The formation of these corrosive materials may even be catalyzed by the presence of such soaps in the oil. Also, some of the metal soaps added as detergents have required the use of free fatty acid and the like to act as a common solvent to promote solution of the soaps in the oil, and the presence of such free acidity has possibly contributed to the corrosion of alloy bearings of the type mentioned above.

Primarily, the object of this invention is to produce for such severe service conditions as are encountered in Diesel engines, lubricating oils which will be non-corrosive to corrosion-sensitive bearings of the copper-lead and cadmium-silver type and which will also avoid the deposition of lacquer and varnish-like materials upon pistons and overcome carbon deposition behind the rings.

The present invention resides in mineral lubricating oils containing small amounts in the order of about 0.5% or 0.75% up to 2% or 3% of oil-soluble metal salts of the weakly acidic non-carboxylic organic acids, said salts being capable

of reacting with acidic corrosive materials formed or present in the oil during use to form metal salts of such corrosion products and liberate free non-carboxylic acids which are sufficiently weak to be non-corrosive to bearings of the copper-lead and cadmium-silver alloy type. It is possible that the metal compounds of weak non-carboxylic organic acids within the scope of this invention also act as anti-oxidants tending to prevent the formation of corrosive acidity.

By the term "weakly acidic non-carboxylic organic acids" it is meant to include those non-carboxylic acidic materials having ionization constants of about  $1 \times 10^{-7}$  or less, and preferably in the range of about  $1 \times 10^{-8}$ , to  $1 \times 10^{-11}$ . However, in some instances it may be acceptable to use materials whose ionization constant is as high as  $1 \times 10^{-6}$ . It may also be possible, at least for some uses, to employ those weakly acidic materials having ionization constants up to about  $5 \times 10^{-6}$ , but in no case so far as now known can about  $5 \times 10^{-6}$  be exceeded; this limit safely excludes the carboxylic acids. Such compounds comprise the phenols, thiophenols, other enols, oximes, sulfonamides having an acidic hydrogen atom, and the like, detailed hereinafter.

Although any of the oil-soluble metal salts of the above mentioned groups of compounds will be effective in preventing the corrosion of bearings such as those of cadmium-silver and copper-lead alloys and will tend to prevent the deposition of carbonaceous materials in the engine, I particularly prefer to employ the oil-soluble metal salts of phenols.

By the term "phenols" it is meant to include not only the hydroxy aromatic ring compounds in which an hydroxyl group is directly attached to a carbocyclic aromatic ring, but also heterocyclic compounds in which the hydroxyl group is attached to a ring containing a sulfur, oxygen, nitrogen or other atom and in which the hydrogen of the hydroxyl group so attached is sufficiently acidic to give the compound an ionization constant within the range defined above, said compound being capable of forming an oil-soluble metal salt. It is to be further understood that the term "phenols" includes not only mono-hydroxy but polyhydroxy compounds and those in which more than one ring is present, such as naphthols and the like. In addition to the hydroxyl group or groups, the ring is preferably substituted by one or more other substituents such as for example, an alkyl group or a sulfur atom linking two phenolic radicals together such as in di-para-tertiary-amyl diphenol sulfide, the

only limits being that the compound must be non-carboxylic, and must contain at least one hydroxyl group of sufficient acidity to exhibit an ionization constant within the limits described above, and must form an oil-soluble metal salt. For the sake of simplicity in the following specification and claims, these compounds will be referred to merely as the metal salts or metal compounds of phenols.

Although it is not definitely known why the metal salts of phenols act to prevent corrosion of alloy bearings and I do not wish to be bound by the theory, it is presumed that this inhibiting power is at least in part connected with the ability of the salts to react with the corrosive acids formed or present in the lubricating oil, to form non-corrosive metal salts of the corrosive acids, thereby liberating the non-corrosive, weakly acidic phenolic compounds. As an indication of the manner in which the above mentioned compounds are presumed to react to neutralize corrosive acidity, thereby rendering the oil non-corrosive, the following exemplary equation may be given:



In this equation R represents a hydrocarbon radical, M represents a metal, X represents the acid radical of a corrosive acid, and H represents a replaceable or acidic hydrogen atom.

All oil-soluble metal salts of phenols, when dissolved in lubricating oil will tend to inhibit the corrosion of bearings of the cadmium-silver and copper-lead type. These include, and I may employ, the oil-soluble Li, Na, K, Cu, Zn, Mg, Ca, Ba, Sr, Al, Pb, Ni, Co, Mn, Cr, Sn and Fe salts of the phenolic compounds. I particularly prefer to employ the alkaline earth salts, calcium, barium, magnesium and strontium, and probably also the aluminum and zinc salts, of the phenolic compounds because of their greater solubility in oil and their possibly lower catalytic activity.

My invention, therefore, resides also in a lubricating oil containing a small amount of an oil-soluble metal compound of a phenolic compound either alone or in combination with other constituents, for example, those adapted to enhance the oiliness or film strength of the oil or even a neutral common solvent, such as the higher boiling alcohol ethers adapted to increase the solubility of the metal salt in the oil.

Also, the invention includes the use of these compounds in lubricating oil in the indicated proportions, in combination with small amounts of other types of oil-soluble soaps having "detergent" properties in the engine in proportion sufficient to overcome or greatly retard the deposition of resinous and varnish-like materials upon piston rings, valves and the like. Such soaps may be used in amounts in the order of 0.5% to 1.0% as required to accomplish the result desired. Such soaps are produced from soap-forming fatty acids and modified fatty acids such as the calcium and magnesium soaps of phenyl stearic acid and chloro stearic acids, and from naphthenic acids, rosin acids, modified rosin acids, and synthetic petroleum acids formed by the oxidation of petroleum fractions such as highly solvent-treated paraffinic type lubricating oil fractions, paraffin waxes, petrolatum and the like. Other metals may be used for soap production, as heretofore indicated, where sufficiently oil soluble soaps are produced.

The mineral lubricating oil employed may be a California or a naphthenic-type oil which ordinarily contains about 0.5% of organically combined sulfur, but may contain as little as 0.15% of such sulfur. Higher sulfur content oils such as those derived from Santa Maria Valley (California), crude oil containing up to 4% or even 5%, for example, 2.75% of such sulfur, are sometimes very desirable. This sulfur also tends to inhibit bearing corrosion and the formation of the acid condition causing it, as elsewhere herein indicated. With metal salts of adequate oil solubility, as in the case of the calcium salts of phenolic compounds containing hydrocarbon side chains attached to the ring, as indicated below, the base may be a well refined paraffinic-type oil.

The oil-soluble metal salts such as the calcium salts of the phenolic compounds are employed in the lubricating oil in amounts up to about 3%, but in amounts less than that required to cause an undesirable thickening of the oil, the optimum apparently being from about 0.5% to 2.0%.

A specific usable phenolic material of which I have produced the calcium salt is di-para-tertiary-butyl diphenol sulfide, which apparently has the formula:



Alkyl hydroxyl phenyl thio ethers of this type are described in the Mikeska et al. Patent No. 2,132,766 and other similar compounds and their method of preparation are given in Mikeska et al. Patent No. 2,139,321.

A phenolic material believed to be kindred to that of the Mikeska et al. Patent No. 2,139,766, is at present obtainable on the market under the trade-name "Paranox" which is available from the Standard Oil Development Company. This material, apparently, is in general composed of mixed poly-alkyl poly-phenol sulfides, that is, poly-alkyl substituted hydroxy phenyl thio ethers containing, for example, a thio ether of butyl phenol which may be designated as Bis (2-hydroxy-4-butyl phenyl) sulfide. This commercial product apparently contains various materials of the following general formulas:



and



In these formulas and similar formulas herein S in general indicates one sulfur atom, but in some molecules two or more sulfur atoms may be represented, the major proportion, however, preferably being monosulfides; R is an alkyl group preferably containing four or five carbon atoms (but may contain more) which groups may be different for the different components of the mixture or may be different for the two or more benzene nuclei in one of the components. R, S and OH may occupy any of the possible positions in the benzene rings. The material may contain higher polymers such as indicated in the second formula above, and even more extensively polymerized materials.

The metal salts of the above described phenolic materials may properly be considered soaps because of an apparent detergent action. When about 1% or between about 0.5% and about 2.0% of such a suitable oil-soluble compound such as

the calcium compound is dissolved in mineral lubricating oil, it has the combined effect of imparting to the mineral lubricating oil where intended for severe service internal combustion engines, the required detergency characteristics and at the same time of acting apparently as a neutralizing agent or, at least in some manner, as an agent for preventing the corrosion of bearings such as those of cadmium-silver and copper-lead alloys.

The invention, therefore, also includes the use of oil-soluble metal salts or compounds of the indicated phenolic type of sulfur-bearing acidic materials, particularly the calcium compounds. It also resides in the use of between about 0.5% and about 3.0% of such soaps in mineral lubricating oils and especially between about 1.0% and about 1.5% of the calcium compounds of the alkyl polyphenol sulfides or polysulfide materials described, especially where the lubricating oils are for use in Diesel engines or other severe service equipment.

In practicing this phase of the invention commercially, the compounds of suitable phenolic compounds such as the calcium compounds of dibutyl or other alkyl or mixtures of alkyl phenol sulfides above indicated may be formed without particular difficulty by any suitable procedure, as will be obvious to the skilled chemist. For example, the calcium salts of these compounds may be conveniently obtained by first adding the starting material to an approximately equal quantity or even greater quantity of a suitable lubricating oil such as a naphthenic base mineral oil having good solvent properties for the phenolic material and for the salts to be produced. This oil mixture is then commingled with hydrated calcium oxide and a small proportion of water, followed by heating to about 300° F. with agitation for a time sufficient to insure neutralization and dehydration. The resultant mixture is filtered to remove solids such as excess calcium oxide. The ash (calcium content) has been increased when desired by first heating only to about 200° F. to 210° F. for a time to insure complete admixture and partial neutralization, the mixture being then cooled to 150° F. to 170° F. and a small quantity in the order of about 3% of 95% alcohol added, and the temperature of the mix then raised to the previously mentioned temperature of 300° F. Another method employed has been to neutralize the alkyl phenol sulfides with sodium hydroxide and then by metathesis with calcium chloride or the like, convert the sodium salt to the calcium salt. In preparing for treatment of the "Paranox" described above as probably comprising a mixture of alkyl phenol sulfides, about 20% of the sulfides should appear in about 80% of lubricating oil having good solvent power for the soap. Otherwise, a greater proportion of lubricating oil is added as its soap-dissolving power decreases. The above described neutralization to produce the calcium salts thereof is more or less easily accomplished due to the fact that the pure phenolic material has been found to have an acid number of about 98. The other alkaline earth metal salts may also be readily produced in a similar manner. In preparing soaps of other metals previously mentioned, the metathesis procedure just mentioned may be preferable as will be readily determined by the skilled chemist.

These salts are readily soluble in lubricating oils in the required proportions and yield alkaline solutions. Representative salts thus pro-

duced appear to have the following structural formulas:



and



In preparing Diesel engine lubricating oil according to the present invention the compound, or the compound-oil mixture, is stirred into an appropriate mineral lubricating oil and solution is effected by agitation, a slight elevation of temperature being produced if desired to facilitate the solution operation.

When the calcium compound is dissolved in the lubricating oil to yield in the final product a compound content in the order of about 1% to 1.5% or in amounts from about 0.5% up to about 3.0%, the detergent action of the resultant lubricating oil is sufficient to overcome or prevent the deposition of the objectionable amounts of said resinous and varnish-like materials above mentioned, and at the same time this quantity of compound is insufficient to substantially increase the original viscosity of the base mineral lubricating oil. Not only do the calcium compounds of these alkyl phenol thio-ethers produce such detergency and thereby prevent sticking of rings and valves and the deposition of varnish-like coatings, but at the same time they prevent the formation of objectionable corrosive acid conditions which attack materially the highly corrosion-sensitive alloy bearings of the copper-lead type.

In addition to the general functions of a compound which are imparted to the oil by this calcium compound, the presence of the sulfur in the compound molecule tends to impart to a non-sulfur-containing lubricating oil, extreme pressure characteristics, and the small percentage of actual sulfur present in the compound further acts to impart in itself some anti-corrosive properties.

In addition to the calcium soaps of the phenol thio-ethers indicated, compounds of other metals of the alkylated phenol thio-ether may be employed such as those of barium and magnesium and also zinc, and aluminum, the important requirements being good solubility in the chosen mineral lubricating oil, detergent properties and freedom from appreciable viscosity increase when used in detergent quantities such as the indicated range from about 0.5 to 2.0%. Also, these metals appear to possess less undesirable catalytic activity than some of the heavier metals previously mentioned such as lead. Compounds of other phenol ethers such as alkyl-substituted phenol selenium or tellurium ethers or the like containing other suitable sulfur substitutes in the ether position are also within the scope of this invention for some uses where possessing sufficient solubility in oil and adequate detergent properties.

I have also found that amyl phenol can be condensed with formaldehyde under appropriate conditions to form a viscous polymer in which free hydroxyl groups of the phenolic type are present. By dissolving this resinous phenolic material in nine volumes of lubricating oil and saponifying by heating with an excess of hydrated lime, followed by dehydration and filtration in the manner described above, I have been able to form the calcium salt of this phenolic resin. When about 1.5% of such a suitable oil-soluble calcium salts was dissolved in mineral lubricating oil it was found to possess the required detergency characteristics and, at the same time, acted to prevent the corrosion of bearings of the cadmium-silver and copper-lead type.

Further, I have found that stearyl alcohol can be condensed with phenol (monohydroxy benzene) in the presence of concentrated sulfuric acid to form a compound believed to be para-stearylphenol. The calcium salt of this compound has likewise been readily formed in the manner described hereinabove and a lubricating oil possessing about 0.65% of the calcium salt of stearylphenol has exhibited the desired detergent and corrosion-preventing properties.

In the foregoing disclosure, the oil-soluble metal compounds of phenolic compounds have been preferred, but it is to be understood that the oil-soluble metal compounds of other weakly acidic, non-carboxylic compounds having ionization constants within the range specified hereinabove are equally satisfactory and are within the scope of the present invention. As group examples of other such weakly acidic, non-carboxylic materials, the phenols, thiophenols, other enols, oximes, sulfonamides and the like were previously mentioned.

The following are specific examples in addition to those given above of suitable acidic materials from the classes just mentioned, and include aryl and alkyl substituted phenols and others of the classes mentioned.

In these instances the designation of the various groups by *m* and *n* is to provide the respective molecules with sufficiently high molecular weights to yield compounds of good solubility in oil. Where the molecule has two rings, it appears that the molecular weight of a compound of good oil-solubility is around 350 or higher. There may be some instances where a compound of as low as 300 molecular weight will be sufficiently oil-soluble, but such apparently is not true of all cases. In general the same lower limits of molecular weights has been taken as representative of compounds of suitable acidic materials of other chemical configuration. Varying values for *m* and *n* also indicate complexity in the molecules, which appears to be a desirable feature imparting greater oil-solubility. Branching appears to promote oil-solubility. Further, mixtures of different molecules in which the alkyl groups vary appear to have better oil-solubility than materials representing a single molecule. Thus, these materials may contain alkyl groups (or aryl groups where indicated) in which *n*, or *m* and *n* combined, may be smaller when the molecules otherwise have relatively high molecular weights, and larger when the molecules otherwise have relatively lower molecular weights. In general it may be said that *m* and *n* will have values from zero to perhaps as high as 20 or possibly higher for molecules otherwise of low molecular weight, and from zero to perhaps about 10 for molecules of otherwise higher molecular weight.

Where different groups appear in the same molecule as indicated by the presence of both *m* and *n*, the number of one will decrease as the other increases at least toward the upper limit, whereby to avoid undesirably high molecular weights.

The following examples of these materials are arranged according to groups above mentioned:

### I. Phenols

#### (a) Monohydroxy phenols

1.



2.



3.



#### (b) Polyhydroxy phenols

1.



(condensation product of p-tert. amylphenol and formaldehyde.)

2.



(As in condensation of oleyl alcohol and phenol)

3.



40 (R may represent groups from propyl to decyl for example.)

4.



50 Here, R represents either an aryl group, such as—



55 or an alkyl group, such as amyl, butyl or other

group between propyl and decyl, or an ester group or the like. Also, at least one R may represent a halogen such as chlorine or other suitable film strength or kindred substituent.

5. Products of the type in all previous examples in which



and the like appear in place of



(c) Condensed ring phenols

1. Products of the type in (a) and (b) above in which



and the like appear in place of



(d) Heterocyclic phenols

1. Compounds of the types in (a), (b), (c) above, in which



and the like appear in place of



## II. Thiophenols

An OH group in the phenol compounds of Group I is replaced with SH.

## III. Oximes

(a)



(b)



(c)



(d)



## IV. Sulfonamides

(a)



(b)



(c)



## V. Imids

(a)



(b)



## VI. Enols

(a)



(b)



Oil-soluble compounds or salts of these various materials may be prepared in manners as outlined above and added in indicated proportions to yield the type of product described and claimed. Important requirements are good solubility of the compounds in oil in the proportions required, without substantial increase in the viscosity of the base oil, and low ionization constants as above defined with consequent freedom from development of corrosive conditions in the oil during engine use which is presumed to be due to the indicated neutralizing character of the compounds which may be termed "reserve alkalinity."

It will be understood that examples are given for purpose of illustration and not as necessarily limiting beyond the requirements of the prior art.

I claim:

65. 1. A lubricant comprising mineral lubricating oil and a small quantity of an oil-soluble metal compound of a thiophenol having an ionization constant in the order about  $1 \times 10^{-7}$  to about  $1 \times 10^{-11}$ , the oil containing also a small proportion of an oil-soluble detergent metal soap of a relatively strong saponifiable carboxylic acid.

2. A mineral lubricating oil for internal combustion engines containing a small proportion of oil-soluble corrosion-controlling metal compound of thiophenol not in itself corrosive to corrosion-

sensitive-alloy bearings, the compound being capable of reacting with strong acidic materials of oxidation produced in the engine to neutralize said strong acidic materials and release said weak organic acids, the oil containing also a small proportion of an oil-soluble detergent metal soap of a relatively strong saponifiable carboxylic acid.

3. A liquid lubricating oil for severe service internal combustion engines comprising mineral lubricating oil containing a small proportion of metal compound of a phenol thioether in quantity sufficient to control development of corrosive conditions without imparting substantial viscosity increase to the base oil, the oil containing also a small proportion of an oil-soluble detergent soap of a saponifiable carboxylic acid.

4. A lubricating oil containing a small proportion of oil-soluble metal compounds of a material from the class consisting of thioenols, the oil also containing a small proportion of an oil-soluble detergent metal soap of a saponifiable organic acid.

5. A mineral lubricating oil for Diesel engines and the like comprising a minor proportion of an oil-soluble detergent metal soap of a saponifiable carboxylic acid, and a minor proportion of an oil-soluble metal salt of an alkylated thio phenolic compound, the salt being capable of neutralizing corrosive conditions developing in an engine.

6. A mineral lubricating oil containing a small proportion between about 0.5% and 3% of an oil-soluble metal salt of an alkylated polyphenol sulfide, and a small proportion in the order of 1% of oil-soluble metal detergent soap of saponifiable organic acids.

7. A liquid mineral lubricating oil for internal combustion engines and the like which comprises a mineral lubricating oil containing in the order of 1% of oil-soluble corrosion-controlling metal salt of a thiophenol having an ionization constant below about  $5 \times 10^{-6}$  and in the order of 1% of oil-soluble metal detergent soap of relatively stronger high molecular weight saponifiable carboxylic acid.

8. A mineral lubricating oil containing a small

proportion in the order of 1% of metal compound of alkylated phenol sulfide, and a small proportion in the order of 1% of a detergent soap of high molecular weight saponifiable carboxylic acid with a metal from the class consisting of alkali metals and heavy metals.

9. A mineral lubricating oil for use in severe service internal combustion engines which contains in the order of 1% of an oil-soluble detergent soap of a saponifiable high molecular weight carboxylic organic acid of the metal of the class consisting of alkali and heavy metals, and between about 0.5% and 3% of a corrosion-controlling metal salt of a weakly acidic thioenolic material.

10. An oil according to claim 9 wherein the corrosion-controlling salt is a salt of an alkylated polyphenol sulfide.

11. An oil according to claim 6 wherein the saponifiable acid is a carboxylic acid.

12. An oil according to claim 6 wherein the saponifiable acid is an acid from the class consisting of fatty acids, modified fatty acids, naphthenic acids, rosin and modified rosin acids, and synthetic acids from the oxidation of petroleum fractions.

13. An oil according to claim 6 wherein the soaps are alkaline earth metal compounds.

14. A freely fluid mineral lubricating oil containing a minor proportion of an oil-soluble metal salt of a phenol sulfide, the oil containing also a small proportion of an oil-soluble detergent metal soap of a relatively strong saponifiable carboxylic acid.

15. An oil according to claim 7 wherein the metal of the thiophenolic salt is from the class consisting of alkali metals and heavy metals.

16. An oil according to claim 14, wherein the metal of the salt of the phenol sulfide is from the class consisting of alkali metals and heavy metals.

17. An oil according to claim 4, wherein the metals of the additives are selected from the class consisting of alkali metals and heavy metals.